

## [54] HEAT DEVELOPABLE PHOTORESITIVE MATERIALS

[75] Inventors: Kageyasu Akashi; Minoru Akiyama; Tetsuo Shiga; Takeki Matsui; Yoshio Hayashi; Takeo Kimura; Hidehiko Kobayashi, all of Fuji, Japan

[73] Assignee: Asahi Kasei Kogyo Kabushiki Kaisha, Tokyo, Japan

[21] Appl. No.: 969,620

[22] Filed: Dec. 14, 1978

## [30] Foreign Application Priority Data

Dec. 23, 1977 [JP] Japan ..... 52-154353  
May 31, 1978 [JP] Japan ..... 53-64241

[51] Int. Cl.<sup>2</sup> ..... G03C 1/02  
[52] U.S. Cl. ..... 430/620; 430/353;  
430/600; 430/613

[58] Field of Search ..... 96/114.1, 109, 66.5,  
96/66.4, 95, 94 R, 94 BF, 66 T, 107

## [56] References Cited

## U.S. PATENT DOCUMENTS

|           |         |                      |          |
|-----------|---------|----------------------|----------|
| 3,457,075 | 7/1969  | Morgan et al. ....   | 96/114.1 |
| 3,689,270 | 9/1972  | Anderson et al. .... | 96/114.1 |
| 3,770,448 | 11/1973 | Poot et al. ....     | 96/114.1 |
| 3,782,941 | 1/1974  | Hartman et al. ....  | 96/114.1 |
| 3,832,186 | 8/1974  | Masuda et al. ....   | 96/114.1 |
| 3,846,136 | 11/1974 | Sullivan ....        | 96/114.1 |
| 3,874,946 | 4/1975  | Costa et al. ....    | 96/114.1 |

|           |         |                       |          |
|-----------|---------|-----------------------|----------|
| 3,877,943 | 4/1975  | Masuda .....          | 96/114.1 |
| 3,885,967 | 5/1975  | Sashihara et al. .... | 96/114.1 |
| 3,951,660 | 4/1976  | Hagemann et al. ....  | 96/114.1 |
| 3,980,482 | 9/1976  | Reece .....           | 96/114.1 |
| 3,997,346 | 12/1976 | Masuda et al. ....    | 96/114.1 |
| 4,003,749 | 1/1977  | Masuda et al. ....    | 96/114.1 |
| 4,009,039 | 2/1977  | Masuda et al. ....    | 96/114.1 |
| 4,021,247 | 5/1977  | Hinata et al. ....    | 96/109   |
| 4,076,539 | 2/1978  | Ikenoue et al. ....   | 96/94 BF |
| 4,120,728 | 10/1978 | Ikenoue et al. ....   | 96/94 BF |
| 4,128,428 | 12/1978 | Ikenoue et al. ....   | 96/114.1 |

Primary Examiner—Travis Brown  
Attorney, Agent, or Firm—Sprung, Felfe, Horn, Lynch & Kramer

[57]

## ABSTRACT

A heat developable photosensitive material comprising:  
(a) an organic silver salt oxidizing agent;  
(b) a halogen molecule or an organic haloamide compound;  
(c) a reducing agent for silver ion; and  
(d) a nitrogen-containing organic base whose pKa of the conjugate acid ranges from 0.5 to 10.0 and the nitrogen-containing organic base having, in its molecule, no acidic proton or a nitrogen-containing organic base whose pKa of its conjugate acid ranges from 0.5 to 10.0 and the nitrogen-containing organic base having, in its molecule, an acidic proton whose pKa is more than 12.

11 Claims, No Drawings

# HEAT DEVELOPABLE PHOTOSENSITIVE MATERIALS

## BACKGROUND OF THE INVENTION

### 1. Field of the Invention

This invention relates to a heat developable photosensitive material. More specifically, it relates to a heat developable photosensitive material having excellent sensitivity and storage stability, which comprises a nitrogen-containing organic base whose conjugate acid has a pKa of from 0.5 to 10.0.

### 2. Description of the Prior Art

Conventional wet processing photosensitive materials using a silver halide emulsion are excellent in their sensitivity, gradation and image quality, but they need complicated time consuming processes using various treating chemicals in obtaining stable images. Further, the chemicals used give rise to a pollution problem. Accordingly, there have been proposed many photosensitive materials capable of forming images thereon easily only by dry processing in a short period of time without using treating chemicals. Such heat developable photosensitive materials use an organic silver salt oxidizing agent as its main component and may be classified into two groups. One is a pre-activation type heat developable photosensitive material on which images can be formed by the imagewise exposure and then the heat development, and the other is a post-activation type heat developable photosensitive material which is non-photosensitive under normal light conditions and can be rendered photosensitive by the preliminary heating prior to the imagewise exposure. For example, the former is described in U.S. Pat. Nos. 3,152,904 and 3,457,075, and the latter is described in U.S. Pat. Nos. 3,802,888 and 3,764,329.

However, the sensitivities of these heat developable photosensitive materials thus proposed are remarkably lower than those of the conventional photosensitive materials containing a silver halide emulsion, and thus utilization of these heat developable photosensitive materials for general purposes are still limited.

## SUMMARY OF THE INVENTION

Extensive investigation have now been made in order to obtain a dry image forming material having excellent sensitivity and storage stability under normal light conditions for practical purposes. These investigations have led to the discovery that a heat developable photosensitive material having remarkably improved properties can be obtained by combining a halogen molecule or an organic haloamide compound as the whole or a part of a compound capable of forming a photosensitive silver compound with a nitrogen-containing organic base whose pKa of the conjugate acid ranges from 0.5 to 10.0.

Accordingly, the present invention provides a heat developable photosensitive material comprising:

- (a) an organic silver salt oxidizing agent;
- (b) a halogen molecule or an organic haloamide compound;
- (c) a reducing agent for silver ion; and
- (d) a nitrogen-containing organic base whose pKa of the conjugate acid ranges from 0.5 to 10.0 and the nitrogen-containing organic base having, in its molecule, no acidic proton or a nitrogen-containing organic base whose pKa of the conjugate acid ranges from 0.5 to 10.0 and the nitrogen-containing

organic base having, in its molecule, an acidic proton whose pKa is more than 12.

## DETAILED DESCRIPTION OF THE INVENTION

In this invention by using the above-described component (d) together with the above-described component (b) as the whole or a part of a component capable of forming a photosensitive silver compound, the sensitivities of the heat developable photosensitive materials of this invention can be remarkably increased without reducing their storage stabilities. This may be presumed that since the heat developable photosensitive materials of this invention comprises a halogen molecule or an organic haloamide compound having a strong oxidability, the use of such a nitrogen-containing organic base can increase their sensitivities without reducing their storage stabilities. When the nitrogen-containing organic base is used together with halogen ion sources other than the halogen molecule or the organic haloamide compound, the sensitivities of the photosensitive materials can be increased but the storage stabilities are remarkably reduced.

The storage stabilities of the heat developable photosensitive materials comprising, in addition to the halogen molecule or the organic haloamide compound, a very strong nitrogen-containing organic base whose conjugate acid has a pKa above 10.0 such as N-methylpiperidine whose conjugate acid has a pKa of 10.1, N-methylpyrrolidine whose conjugate acid has a pKa of 10.4 and pyrrolidine whose conjugate acid has a pKa of 11.3 are low. Also the sensitivities of the heat developable photosensitive materials comprising, in addition to the halogen molecule or the organic haloamide compound, a weak nitrogen-containing organic base whose conjugate acid has a pKa below 0.5 such as 2-fluoropyridine whose conjugate acid has a pKa of 0.4 can hardly be increased.

According to this invention in case where the nitrogen-containing organic base has an acidic proton in its molecule even when the pKa of the conjugate acid of the nitrogen-containing organic base ranges from 0.5 to 10.0, an anti-fogging effect by the acidic component appears at the same time. When the pKa of an acidic proton is more than 12 as with benzimidazole or pyrazole, the effect by the acidic component hardly appears as with the nitrogen-containing organic base having no acidic proton in its molecule. However, when the pKa of an acidic proton is 12 or less than 12 as with benztriazole or tetrazole, the storage stability of the photosensitive material is not reduced but the increase in its sensitivity is small.

The nitrogen-containing organic bases whose conjugate acids have a pKa of from 0.5 to 10.0 which can be employed as component (d) in the heat developable photosensitive material of this invention include pyridine, quinoline, isoquinoline, acridine, phenanthridine, pyridazine, pyrimidine, pyrazine, cinnoline, phthalazine, quinazoline, quinoxaline, phenazine, m-, o-, p-phenanthroline, pteridine, pyrazole, imidazole, benzimidazole; derivatives thereof having a substituent such as an alkyl group, a substituted alkyl group, an aryl group, a substituted aryl group, a nitro group, a halogen atom, a nitrile group, an alkoxy group or a carboxyalkyl group.

Specific examples of such derivatives include 2-chloropyridine, 3-chloropyridine, 2-bromopyridine,

3-bromopyridine, 2-methylpyridine, 3-methylpyridine, 4-methylpyridine, 2,6-diisopropylpyridine, 2-isopropylpyridine, 2-tertbutylpyridine, 3-phenylpyridine, 2,6-di-tert-butylpyridine, 3-acetylpyridine,  $\alpha, \alpha'$ -dipyridyl,  $\beta, \beta'$ -dipyridyl,  $\gamma, \gamma'$ -dipyridyl, 5-nitro-1,10-phenanthroline, 2-methylquinoline, 3-methylquinoline, 4-methylquinoline, 2-chloroquinoline, 4-chloroquinoline, 2-methoxyisoquinoline, 4-methylpyrimidine, 2-dimethylaminopyrimidine, 2-methoxyquinazoline, 2-methylquinoxaline, 1-methylpyrazole and 2-methylpyrazole.

Of these nitrogen-containing organic bases, 6-membered ring nitrogen-containing organic bases such as pyridine, quinoline, isoquinoline, pyrazine, phthalazine, quinoxaline, quinazoline, cinnoline, pyridazine and pyrimidine which are comparatively stable against the oxidation by the halogen molecule or the organic haloamide compound as component (b) in the heat developable photosensitive material of this invention are preferred due to their ease in handling.

The amount of the nitrogen-containing organic base typically ranges from about 0.001 mole to about 1 mole, and preferably from about 0.01 mole to about 0.5 mole per mole of the organic silver salt oxidizing agent.

The pKa and the method of measuring the same which are used in this invention are described in Adrien Albert, "Heterocyclic Chemistry, an Introduction", published by Athlone Press, University of London in 1959; Chemical Society of Japan, "Kagaku Binran (Chemical Dictionary)", published by Maruzen 1966; and E. J. King, "Acid-Base Equilibria", published by Pergamon Press, New York in 1965.

The organic silver salt oxidizing agents which can be employed as component (a) in this invention include silver salts of long chain aliphatic carboxylic acids having 12 to 24 carbon atoms such as silver laurate, silver myristate, silver palmitate, silver stearate, silver arachidate and silver behenate, silver salts of organic compounds having an imino group such as benztriazole silver salt, benzimidazole silver salt, carbazole silver salt and phthalazinone silver salt; silver salts of sulfur containing compounds such as S-alkylthioglycollates; silver salts of aromatic carboxylic acids such as silver benzoate and silver phthalate; silver salts of sulfuric acids such as silver ethanesulfonate; silver salts of sulfonic acids such as silver o-toluenesulfonate; silver salts of phosphoric acids such as silver phenylphosphate; silver barbiturate; silver saccharate; silver salts of salicylaldoxime; and any mixtures thereof. Of these compounds, the silver salts of long chain aliphatic carboxylic acids having 12 to 24 carbon atoms are preferred.

The amount of the organic silver salt oxidizing agent which can be employed in this invention typically ranges from about 0.1 g/m<sup>2</sup> to about 50 g/m<sup>2</sup> of the support area of the heat developable photosensitive material. A preferred amount of the organic silver salt oxidizing agent ranges from about 1 g/m<sup>2</sup> to about 10 g/m<sup>2</sup> of the support area of the heat developable photosensitive material.

The halogen molecules which can be employed as component (b) in this invention include iodine molecule, bromine molecule, iodine monochloride and iodine trichloride, iodine bromide and bromine chloride. The bromine chloride is preferably used in the form of a hydrate which is solid.

The term "halogen molecule" used herein includes not only the above-described halogen molecules but also complexes of a halogen molecule, for example, complexes of a halogen molecule with p-dioxane which

are generally solid. Of the halogen molecules that can be used in this invention, iodine molecule which is solid under normal conditions is especially preferred.

The organic haloamide compounds which can be employed as component (b) in this invention include, for example, N-chlorosuccinimide, N-bromosuccinimide, N-iodosuccinimide, N-chlorophthalimide, N-bromophthalimide, N-iodophthalimide, N-chlorophthalazinone, N-bromophthalazinone, N-iodophthalazine, N-chloroacetamide, N-bromoacetamide, N-iodoacetamide, N-chloroacetanilide, N-bromoacetanilide, N-iodoacetanilide, 1-chloro-3,5,5-trimethyl-2,4-imidazolidinedione, 1-bromo-3,5,5-trimethyl-2,4-imidazolidinedione, 1-iodo-3,5,5-trimethyl-2,4-imidazolidinedione, 1,3-di-chloro-5,5-dimethyl-2,4-imidazolidinedione, 1,3-dibromo-5,5-dimethyl-2,4-imidazolidinedione, N,N-dichlorobenzenesulfonamide, N,N-dibromobenzenesulfonamide, N-bromo-N-methylbenzenesulfonamide, N-chloro-N-methylbenzenesulfonamide, N,N-diiodobenzenesulfonamide, N-iodo-N-methylbenzenesulfonamide, 1,3-dichloro-4,4-dimethylhydantoin, 1,3-dibromo-4,4-dimethylhydantoin and 1,3-diiodo-4,4-dimethylhydantoin.

In general, the halogen molecules are more effective for improving both the sensitivity and the storage stability of the photosensitive materials than the organic haloamide compounds. The amount of the halogen molecules or the organic haloamide compounds typically ranges from about 0.001 mole to about 0.5 mole, and preferably from about 0.01 mole to about 0.2 mole, based on the mole of the organic silver salt oxidizing agent.

In order to further increase the sensitivity of the heat developable photosensitive materials of this invention without sacrifice of their storage stability, another halogen ion sources may be used together with the above-mentioned halogen molecule or the above-mentioned organic haloamide compound.

As the halogen ion source in the photosensitive material of this invention, any of compounds capable of generating a halogen ion may be used. Examples of such halogen ion sources include calcium iodide, barium iodide, rubidium iodide, cesium iodide, aluminum iodide, magnesium iodide, sodium iodide, potassium iodide, bromides and chlorides corresponding to the above-mentioned iodides, and quaternary tetraalkyl ammonium salts such as tetraethyl ammonium salts, quaternary aralkyl trialkyl ammonium salts such as benzyl trimethyl ammonium salts and quaternary aryl trialkyl ammonium salts such as phenyl trimethyl ammonium salts, said quaternary ammonium salts being those of hydroiodic acid, hydrobromic acid and hydrochloric acid. Further examples of the halogen ion source include ionizable organic halogen compounds such as triphenylmethyl iodide and phenacyl bromide; nonmetallic halogen compounds such as triphenylphosphine diiodide, triphenylphosphine dibromide, triphenylphosphite diiodide and triphenylphosphite dibromide; halogen-containing organometallic compounds such as titanocene dichloride, zirconocene dichloride, dimethylsilyl dichloride, trimethylsilyl chloride and triphenylgermanium bromide. These compounds to be used as the halogen ion source may be used alone or in combination. The amount of the halogen ion source to be used may be about 0.1 to about 20 mole %, preferably about 0.5 to 10 mole %, based on the amount of the organic silver salt oxidizing agent.

The halogen ion source and the halogen molecule may be added separately, or a compound or compounds capable of forming a halogen ion source and a halogen molecule by reaction at the preparation of the photosensitive material may be used. Following is an explanation of the illustrate mode of use of a combination of the halogen ion source and an iodine molecule in the form of a compound or compounds described above. The explanation is made exemplifying the use of iodine as the halogen. For example, triphenylphosphite diiodide and iodine molecule can be formed by the use of triphenyl phosphite and an excessive amount of molecular iodine. Also, triphenylphosphite nonaiodide as synthesized according to the method disclosed in J. Am. Chem. Soc., 75, p. 3145 (1953) is dissociated into triphenylphosphite diiodide and molecular iodine at the time of preparation of the composition for the heat developable photosensitive material, even when it is used alone. When this triphenylphosphite nonaiodide is employed, there is obtained a photosensitive material having good storage stability and good sensitivity, and hence, the use of triphenylphosphite nonaiodide is preferred.

As exemplary combinations of the compounds, there can be mentioned combinations of molecular iodine and phosphites such as alkyl phosphites, e.g., tributyl phosphites and tristearyl phosphite, and aryl phosphites, e.g., triphenyl phosphite and tricresyl phosphites; combination of molecular iodine and phosphines such as triphenylphosphine; combination of molecular iodine and tellurides such as dibutyltelluride and diphenyl telluride; combination of molecular iodine and arsines such as triphenylarsine and tributylarsine.

The above explanation is made with respect to the case where iodine is used as a halogen molecule, but the similar combinations may be used with respect to the case of other halogen molecules.

The reducing agents for silver ion which can be used as component (c) in this invention include sterically hindered phenols in which a sterically bulky group is bonded to the carbon atom adjacent to the carbon atom bonded to the hydroxyl group; substituted phenols; hydroquinones; hydroquinone ethers; and other reducing agents for conventional wet processing silver salt type photosensitive materials.

Specific examples of such reducing agents for silver ion include 2,6-di-tert-butyl-4-methylphenol, 2,2'-methylenebis(4-methyl-6-tertbutylphenol), 2,6-methylenebis(2-hydroxy-3-tert-butyl-5-methylphenyl)4-methylphenol, 2,2'-methylenebis(4-ethyl-6-tert-butylphenol), 2,6-bis(2'-hydroxy-3'-tert-butyl-5'-methylbenzyl)4-methylphenol, 2,4,4-trimethylpentyl-bis(2-hydroxy-3,5-dimethylphenyl)methane, 2,2'-methylenebis[4-methyl-6-(1-methylcyclohexyl)]phenol, 2,5-di-tert-butyl-4-methoxyphenol; p-phenylphenol, p-methoxyphenol, p-aminophenol, catechol, pyrogallol, resorcin, bisphenol A, 2,4-dihydroxybenzoic acid; hydroquinone, chlorohydroquinone, bromohydroquinone, phenylhydroquinone, methylhydroquinone, tert-butylhydroquinone, tert-octylhydroquinone, 2,5-dimethylhydroquinone, 2,6-dimethylhydroquinone, methoxyhydroquinone; hydroquinone monobenzyl ether;  $\alpha$ -naphthol,  $\beta$ -naphthol, 1,3-dihydroxynaphthalene, 2,2'-dihydroxy-1,1'-binaphthyl; phenidone, methyl gallate; and any mixtures thereof.

A preferred reducing agent for silver ion can be chosen depending upon the organic salt oxidizing agent employed. For example, with an organic silver salt

oxidizing agent such as silver behenate which is relatively hard to be reduced, a relatively strong reducing agent for silver ion such as a sterically hindered phenol including 2,2'-methylenebis(4-ethyl-6-tert-butylphenol) is suitably chosen. On the other hand, with an organic silver salt oxidizing agent such as silver laurate which is relatively easy to be reduced, a relatively weak reducing agent for silver ion such as a substituted phenol including p-phenylphenol is suitably chosen, and with an organic silver salt oxidizing agent such as silver salt of benztriazole which is very hard to be reduced, a strong reducing agent for silver ion such as ascorbic acid is suitably chosen.

The amount of the reducing agent for silver ion may vary depending upon the organic silver salt oxidizing agent selected. In general, the amount of the reducing agent for silver ion used ranges from about 0.1 percent by weight to about 200 percent by weight based on the weight of the organic silver salt oxidizing agent. A preferred amount of the reducing agent for silver ion ranges from about 1 percent by weight to about 100 percent by weight.

If necessary or if desired, the heat developable photosensitive materials of this invention may further comprise conventional modifiers such as a binder for film formation, a toner for silver images, an antifoggant and a background-darkening preventing agent in addition to the above-described components (a), (b), (c) and (d).

The binder is needed for film formation in many cases.

As exemplary film-forming binders, there can be mentioned polyvinyl acetate, vinyl chloride-vinyl acetate copolymers, polyvinyl chloride, polyvinyl butyral, polymethyl methacrylate, cellulose acetate, cellulose acetate propionate, cellulose acetate butyrate, polyvinyl alcohol, polyvinyl pyrrolidone, gelatin and polystyrene. They may be used along or in mixture. The film-forming binder can be used generally in such an amount that the weight ratio of the binder to the organic silver salt oxidizing agent is in the range of from about 0.1 to about 10. As the toner for a silver image, there can be mentioned, for example, phthalazinone, maleic hydrazide, benzoxazidinedione, cyclic imides, quinazolinone, 2-pyrazoline-5-one, zinc acetate and cadmium acetate. The toner may be used suitably in an amount of 0.01 to 1 mole per mole of the organic silver salt oxidizing agent.

In this invention, a practically useful photosensitive material can be prepared even if an anti-foggant is not particularly added. If a higher anti-foggant effect is required, an anti-foggant may, of course, be used in this invention. As the anti-foggant, there can be mentioned mercury salts, palladium salts, and a wide variety of acidic compounds. For example, when mercuric acetate is used as the anti-foggant in an amount as small as about 0.01 mole % based on the amount used of the organic silver salt oxidizing agent, a remarkable anti-foggant effect can be attained in the photosensitive material of this invention.

As the background-darkening preventing agent, there can be mentioned, for example, tetrabromobutane and hexabromocyclohexane. This agent may be used suitably in an amount of from about 2.5 to about 14 mole % based on the organic silver salt oxidizing agent.

A preferred method of preparing the heat developable photosensitive material of this invention is described by way of example as follows. An organic silver salt oxidizing agent as prepared separatively is dispersed

in a binder solution or emulsion for a photographic emulsion by means of a sand grinder, a mixer, a ball mill or the like. To the resulting dispersion are, in turn, added additives such as a halogen molecule, a reducing agent and the like. The composition thus obtained is applied onto a support such as a plastic film, a glass plate, a paper or a metal plate to prepare a photosensitive material. As the plastic film, there can be mentioned, for example, cellulose triacetate and other cellulose acetate films, polyethylene terephthalate and other polyester films, polyamide films, polyimide films, a polyvinyl acetal film, a polystyrene film, a polyethylene film and polycarbonate films. As the paper, there can be mentioned, for example, a photographic base paper, a coated paper, an art paper and a barite paper and a 15 water-proof paper as well as ordinary papers. An aluminum plate can be used as a metal plate by way of example.

The dry thickness of the coating is from about 1 to about  $1,000\mu$ , preferably from about 3 to about  $20\mu$ . 20 The ingredients of the composition may be applied and laminated separately in two or more layers, optionally. The sheet material thus prepared is non-photosensitive under normal lighting conditions and it can be handled in a light room. When a given area of this sheet material is heated in the dark, this area is rendered photosensitive. This preliminary heating is preferably carried out at a temperature of about  $90^\circ$  to about  $200^\circ$  C. If the heating temperature is elevated, the heating time may be proportionally short. When the area rendered photosensitive by heating is exposed imagewise to light and then heat-developed, a visible image is obtained. It is preferred that heat development be carried out at a temperature of about  $90^\circ$  to about  $200^\circ$  C. The heating period of time at either the preliminary heating or the 35 heat development may be controlled within the range of from about 1 to about 60 seconds. When the preliminary heating for rendering the material photosensitive and the heat development are conducted at the same temperature, the time for the heat development is generally longer than the time for the preliminary heating. With the heat developable photosensitive materials of this invention, a visible image can be recorded selectively on a given area, and up-dated information may be additionally recorded on other areas according to need. 45

The present invention will now be illustrated in more detail by the following non-limiting examples.

#### EXAMPLE 1

To 20 parts by weight of a mixed liquid of methyl 50 ethyl ketone and toluene in a weight ratio of 2 to 1 were

added 4 parts by weight of silver behenate, and the mixture was ball-milled for about 24 hours to give a uniform silver behenate suspension.

Then, an emulsion having the first layer composition as set forth below was prepared by mixing each of its ingredients in the order described therein with stirring and coated on a polyester film as the first layer, and then dried. The thickness of the first layer was  $4\mu$ .

| First Layer Composition                                               |        |
|-----------------------------------------------------------------------|--------|
| Silver behenate suspension                                            | 12.0 g |
| Polyvinyl butyral                                                     | 3.0 g  |
| Methyl ethyl ketone                                                   | 12.0 g |
| Mercuric acetate                                                      | 0.05 g |
| Iodine molecule                                                       | 0.12 g |
| Nitrogen-containing organic base in an amount as set forth in Table 1 |        |

Then, another solution having the second layer composition as set forth below was prepared and coated on the first layer as the second layer, and then dried. The total thickness of the first and second layer was  $7\mu$ .

| Second Layer Composition                      |        |
|-----------------------------------------------|--------|
| Cellulose acetate                             | 1.2 g  |
| Acetone                                       | 16.3 g |
| Phthalazinone                                 | 0.28 g |
| 2,2'-Methylenebis(6-tert-butyl-4-ethylphenol) | 0.70 g |

Each of the photosensitive materials thus obtained which were non-photosensitive under normal light conditions was preliminarily heated at  $100^\circ$  C. for 5 seconds in a dark room, and then exposed to light from a 500 watt xenon lamp for one eighth of second through a mask film and subsequently heated at  $130^\circ$  C. for 1 second to develop a negative image.

The maximum optical densities and the minimum optical densities of the images thus obtained are shown in Table 1.

Further, each of the photosensitive materials was kept at  $50^\circ$  C. at a relative humidity of 90% for 24 hours in a dark room prior to the preliminary heating in order to test its storage stability, and subsequently an image was formed thereon in the same manner as described above.

The maximum optical densities and the minimum optical densities of the images thus obtained are also shown in Table 1.

Table 1

| Run No. | Organic Base (g)   | Nitrogen-containing Organic Base | pKa of Conjugate Acid | Optical Density of Image |         |          |          |
|---------|--------------------|----------------------------------|-----------------------|--------------------------|---------|----------|----------|
|         |                    |                                  |                       | Maximum                  | Minimum | Maximum* | Minimum* |
| 1       | Pyridine           | 0.30                             | 5.2                   | 1.88                     | 0.06    | 1.83     | 0.07     |
| 2       | Quinoline          | 0.30                             | 4.9                   | 2.55                     | 0.06    | 2.50     | 0.06     |
| 3       | Isoquinoline       | 0.30                             | 5.4                   | 2.63                     | 0.07    | 2.54     | 0.07     |
| 4       | Phthalazine        | 0.05                             | 3.5                   | 2.23                     | 0.06    | 2.30     | 0.06     |
| 5       | Quinazoline        | 0.60                             | 3.5                   | 2.41                     | 0.06    | 2.13     | 0.07     |
| 6       | Pyrazine           | 0.03                             | 6.0                   | 1.96                     | 0.07    | 1.90     | 0.08     |
| 7       | Pyridazine         | 0.30                             | 2.3                   | 1.55                     | 0.06    | 1.48     | 0.08     |
| 8       | Pyrimidine         | 0.30                             | 1.3                   | 2.20                     | 0.08    | 1.21     | 0.09     |
| 9       | Quinoxaline        | 0.60                             | 0.7                   | 1.90                     | 0.06    | 1.90     | 0.06     |
| 10      | Cinnoline          | 0.30                             | 2.3                   | 1.92                     | 0.06    | 1.89     | 0.07     |
| 11      | Pyrazole           | 0.05                             | 2.5                   | 2.38                     | 0.07    | 2.44     | 0.09     |
| 12      | N-Ethyl-morpholine | 0.10                             | 7.6                   | 1.89                     | 0.08    | 1.85     | 0.09     |
| 13      | Piperazine         | 0.10                             | 9.8                   | 1.78                     | 0.09    | 1.76     | 0.10     |

Table 1-continued

| Run No.            | Nitrogen-containing Organic Base (g) | pKa of Conjugate Acid | Optical Density of Image |         |          |          |
|--------------------|--------------------------------------|-----------------------|--------------------------|---------|----------|----------|
|                    |                                      |                       | Maximum                  | Minimum | Maximum* | Minimum* |
| <b>Comparative</b> |                                      |                       |                          |         |          |          |
| 1                  | None                                 | —                     | 0.34                     | 0.06    | 0.17     | 0.07     |
| 2                  | N-Methyl-piperidine                  | 0.10                  | 10.1                     | 1.88    | 0.10     | 1.79     |
| 3                  | N-Methyl-pyrrolidine                 | 0.10                  | 10.4                     | 1.75    | 0.11     | 1.70     |
| 4                  | Pyrrolidine                          | 0.05                  | 11.3                     | 1.83    | 0.10     | 1.66     |
| 5                  | Azetidine                            | 0.10                  | 11.3                     | 1.83    | 0.10     | 1.83     |

\*The image was formed on the photosensitive material after the storage stability test.

### EXAMPLE 2

The same procedures as described in Run Nos. 1 to 5 and Comparative Run No. 1 of Example 1 were re-

The maximum optical densities and the minimum optical densities of the image thus formed and those of the images formed after the same storage stability test as in Example 1 are shown in Table 3 below.

Table 3

| Run No.            | Nitrogen-containing Organic Base (g) | Optical Density of Image |         |          |          |      |
|--------------------|--------------------------------------|--------------------------|---------|----------|----------|------|
|                    |                                      | Maximum                  | Minimum | Maximum* | Minimum* |      |
| 1                  | Pyridine                             | 0.30                     | 1.38    | 0.06     | 1.21     |      |
| 2                  | Quinoline                            | 0.30                     | 1.29    | 0.06     | 1.30     |      |
| 3                  | Isoquinoline                         | 0.30                     | 1.41    | 0.06     | 1.38     |      |
| 4                  | Phthalazine                          | 0.30                     | 1.63    | 0.07     | 1.64     |      |
| 5                  | Quinazoline                          | 0.30                     | 1.32    | 0.06     | 1.33     |      |
| <b>Comparative</b> |                                      |                          |         |          |          |      |
| Run No.            |                                      |                          |         |          |          |      |
| 1                  | None                                 | —                        | 0.23    | 0.06     | 0.21     | 0.07 |

\*The image was formed on the photosensitive material after the same storage stability test as in Example 1.

peated except that 0.28 g of phthalimide was used instead of the phthalazinone and that 0.70 g of 2,6-bis(2'-hydroxy-3'-tert-butyl-5'-methylbenzyl)-4-methylphenol was used instead of the 2,2'-methylenebis(6-tert-butyl-4-ethylphenol).

The maximum optical densities and the minimum optical densities of the images thus formed and those of the images formed after the same storage stability test as in Example 1 are shown in Table 2 below.

### EXAMPLE 4

The same procedures of producing photosensitive materials as described in Run Nos. 1 to 3 and Comparative Run No. 1 of Example 1 were repeated except that 0.12 g of the complex of bromine with p-dioxane was used instead of the iodine molecule.

Each of the photosensitive materials thus obtained was preliminarily heated at 110° C. for 3 seconds in a

Table 2

| Run No.            | Nitrogen-containing Organic Base (g) | Optical Density of Image |         |          |          |      |
|--------------------|--------------------------------------|--------------------------|---------|----------|----------|------|
|                    |                                      | Maximum                  | Minimum | Maximum* | Minimum* |      |
| 1                  | Pyridine                             | 0.30                     | 1.77    | 0.06     | 1.76     |      |
| 2                  | Quinoline                            | 0.30                     | 1.86    | 0.06     | 1.79     |      |
| 3                  | Isoquinoline                         | 0.30                     | 1.63    | 0.07     | 1.58     |      |
| 4                  | Phthalazine                          | 0.10                     | 1.80    | 0.06     | 1.75     |      |
| 5                  | Quinazoline                          | 0.20                     | 1.71    | 0.06     | 1.80     |      |
| <b>Comparative</b> |                                      |                          |         |          |          |      |
| Run No.            |                                      |                          |         |          |          |      |
| 1                  | None                                 | —                        | 0.22    | 0.06     | 0.20     | 0.07 |

\*The image was formed on the photosensitive material after the same storage stability test as in Example 1.

### EXAMPLE 3

The same procedure as described in Run Nos. 1 to 5 and Comparative Run No. 1 of Example 1 were repeated except that 0.28 g of maleic hydrazide was used instead of the phthalazinone.

dark room, and then exposed to light from a 300 watt tungsten lamp for one eighth of second through a mask film and subsequently heated at 130° C. for 3 seconds to develop a negative image.

The maximum optical densities and the minimum optical densities of the image thus formed and those of the images formed after the same storage stability test as in Example 1 are shown in Table 4 below.

Table 4

| Run No.             | Nitrogen-containing Organic Base (g) | Optical Density of Image |         |          |          |
|---------------------|--------------------------------------|--------------------------|---------|----------|----------|
|                     |                                      | Maximum                  | Minimum | Maximum* | Minimum* |
| 1                   | Pyridine                             | 0.30                     | 1.11    | 0.06     | 1.03     |
| 2                   | Quinoline                            | 0.30                     | 1.09    | 0.06     | 1.04     |
| 3                   | Isoquinoline                         | 0.30                     | 0.99    | 0.07     | 1.00     |
| Comparative Run No. |                                      |                          |         |          |          |
| 1                   | None                                 | —                        | 0.22    | 0.05     | 0.18     |
|                     |                                      |                          |         | 0.07     |          |

\*The image was formed on the photosensitive material after the same storage stability test as in Example 1.

### COMPARATIVE EXAMPLE 1

The same procedures as described in Run Nos. 1 to 3 and Comparative Run No. 1 of Example 1 were repeated except that 0.10 g of ammonium bromide was used instead of the iodine molecule and that the preparation of the heat developable photosensitive materials was conducted in a dark room.

The maximum optical densities and the minimum optical densities of the images thus formed and those of the images formed after the same storage stability test as in Example 1 are shown in Table 5 below.

Table 5

| Run No.             | Nitrogen-containing Organic Base (g) | Optical Density of Image |         |          |          |
|---------------------|--------------------------------------|--------------------------|---------|----------|----------|
|                     |                                      | Maximum                  | Minimum | Maximum* | Minimum* |
| 1                   | Pyridine                             | 0.30                     | 2.30    | 0.07     | 2.21     |
| 2                   | Quinoline                            | 0.30                     | 2.06    | 0.06     | 2.06     |
| 3                   | Isoquinoline                         | 0.30                     | 2.11    | 0.06     | 2.06     |
| Comparative Run No. |                                      |                          |         |          |          |
| 1                   | None                                 | —                        | 0.11    | 0.06     | 0.12     |
|                     |                                      |                          |         | 0.06     |          |

\*The image was formed on the photosensitive material after the same storage stability test as in Example 1.

### EXAMPLE 5

An emulsion having the composition as set forth below was prepared by mixing each of its ingredients in the order described therein with stirring and coated on a sheet of art paper, and then dried in air.

| Composition                                                                       |          |
|-----------------------------------------------------------------------------------|----------|
| The same silver behenate suspension as in Example 1                               | 45 1.5 g |
| Methyl ethyl ketone solution containing 14 percent by weight of polyvinyl butyral | 1.2 g    |
| Mercuric acetate                                                                  | 1 mg     |
| Iodine bromide                                                                    | 14 mg    |
| Nitrogen-containing organic base as shown below*                                  | 30 mg    |
| Phthalazinone                                                                     | 30 mg    |
| 2,2'-Methylenebis(6-tert-butyl-4-ethylphenol)                                     | 70 mg    |

- \*(1) Quinoline
- (2) Isoquinoline
- (3) 1-Methylpyrrolidinone
- (4) 1-Methylpyridone
- (5) None

Each of the photosensitive materials thus obtained was preliminarily heated at 100° C. for 4 seconds in a dark room and then exposed to light from a 150 watt xenon lamp for one fifth of second through a mask film, and subsequently heated at 120° C. for 6 seconds to develop a negative image.

The photosensitive material containing the quinoline or the isoquinoline as a nitrogen-containing organic base gave a very clear dark image with high contrast. On the other hand, the photosensitive material without

the nitrogen-containing organic base or containing the 1-methylpyrrolidinone or the 1-methylpyridone gave a light brown with very low contrast.

### EXAMPLE 6

A benztriazole silver suspension was prepared in the same manner as described in Example 1 except that the same amount of benztriazole silver salt as the silver behenate was used instead of the silver behenate.

An emulsion having the composition as set forth below was prepared by mixing each of its ingredients in the order described therein with stirring and coated on

a sheet of paper, and then dried.

| Composition                    |         |
|--------------------------------|---------|
| Benztriazole silver suspension | 12.0 g  |
| Polyvinyl butyral              | 2.5 g   |
| Methyl ethyl ketone            | 12.0 g  |
| Mercuric acetate               | 0.025 g |
| Iodine molecule                | 0.12 g  |
| Phthalazinone                  | 0.25 g  |
| Tert-butylhydroquinone         | 0.40 g  |
| Quinoline                      | 0.40 g  |

The photosensitive material thus obtained was preliminarily heated at 100° C. for 5 seconds with a hot roll in a dark room and then exposed to light from a 1 KW photograph lamp for one thirtieth of second through a mask film, followed by heat development at 130° C. for 2 minutes. The image thus obtained was very dark and clear. On the other hand, the image formed on the photosensitive material containing no quinoline was barely observed in light brown color.

### EXAMPLE 7

An emulsion having the first layer composition as set forth below was prepared by mixing each of its ingredients in the order described therein with stirring and coated on a polyester film and then dried.

| First Layer Composition                             |           |
|-----------------------------------------------------|-----------|
| The same silver behenate suspension as in Example 1 | 65 12.0 g |
| Polyvinyl butyral                                   | 3.0 g     |

-continued

| First Layer Composition                                               |        |
|-----------------------------------------------------------------------|--------|
| Methyl ethyl ketone                                                   | 12.0 g |
| Mercuric acetate                                                      | 0.05 g |
| Diphenyltellurium dibromide                                           | 0.05 g |
| Iodine molecule                                                       | 0.10 g |
| Nitrogen-containing organic base<br>in an amount as shown in Table 6. |        |

Then, another solution having the second layer composition as set forth below was prepared and coated on the first layer as the second layer, and then dried.

| Second Layer Composition |  |
|--------------------------|--|
|                          |  |

14 watt tungsten lamp for one sixtieth of second through a mask film and subsequently heated at 120° C. for 3 seconds to develop a negative image.

5 The maximum optical densities and the minimum optical densities of the images thus obtained are shown in Table 6.

Further, each of the photosensitive materials was kept at 60° C. at a relative humidity of 90% for one hour in a dark room prior to the preliminary heating in order 10 to test its storage stability, and subsequently an image was formed thereon in the same manner as described above.

15 The maximum optical densities and the minimum optical densities of the images thus obtained are also shown in Table 6.

Table 6

| Run<br>No.             | Nitrogen-<br>containing<br>Organic Base<br>(g) | pKa<br>of<br>Conjugate<br>Acid | Optical Density of Image |         |          |          |      |
|------------------------|------------------------------------------------|--------------------------------|--------------------------|---------|----------|----------|------|
|                        |                                                |                                | Maximum                  | Minimum | Maximum* | Minimum* |      |
| 1                      | Quinoline                                      | 0.30                           | 4.9                      | 1.99    | 0.07     | 1.81     | 0.07 |
| 2                      | 2-Methyl-<br>quinoline                         | 0.30                           | 5.4                      | 1.86    | 0.06     | 1.85     | 0.06 |
| 3                      | 5-Methyl-<br>quinoline                         | 0.30                           | 4.6                      | 1.90    | 0.06     | 1.91     | 0.06 |
| 4                      | 3-Chloro-<br>quinoline                         | 0.30                           | 2.4                      | 1.60    | 0.06     | 1.43     | 0.06 |
| 5                      | Pyridine                                       | 0.30                           | 5.2                      | 1.47    | 0.07     | 1.30     | 0.07 |
| 6                      | α,α'-Dipyridyl                                 | 0.15                           | 4.4                      | 1.88    | 0.06     | 1.87     | 0.06 |
| 7                      | α,α'-Nitro-1,10-<br>phenanthroline             | 0.30                           | 3.75                     | 1.55    | 0.08     | 1.51     | 0.09 |
| 8                      | 2-Tert-butyl-<br>pyridine                      | 0.30                           | 5.8                      | 2.01    | 0.07     | 2.10     | 0.08 |
| 9                      | 2,6-Diisopropyl-<br>pyridine                   | 0.30                           | 5.3                      | 1.97    | 0.06     | 2.10     | 0.09 |
| 10                     | 3-Acetylpyridine                               | 0.30                           | 3.2                      | 1.68    | 0.07     | 1.56     | 0.07 |
| 11                     | Pyrimidine                                     | 0.30                           | 1.3                      | 1.54    | 0.08     | 1.44     | 0.08 |
| 12                     | 4-Methyl-<br>pyrimidine                        | 0.20                           | 2.0                      | 1.73    | 0.08     | 1.74     | 0.08 |
| 13                     | Phthalazine                                    | 0.10                           | 3.5                      | 2.25    | 0.06     | 2.20     | 0.06 |
| 14                     | Pyrazole                                       | 0.10                           | 2.5                      | 1.58    | 0.07     | 1.50     | 0.09 |
| 15                     | 3-Methyl-<br>pyrazole                          | 0.10                           | 3.6                      | 1.90    | 0.06     | 2.00     | 0.09 |
| Comparative<br>Run No. |                                                |                                |                          |         |          |          |      |
| 1                      | None                                           | —                              | —                        | 0.20    | 0.06     | 0.18     | 0.08 |
| 2                      | Benztriazole**                                 | 0.30                           | 1.6                      | 0.53    | 0.06     | 0.48     | 0.06 |
| 3                      | Tetrazole***                                   | 0.30                           | —                        | 0.42    | 0.05     | 0.36     | 0.06 |
| 4                      | 1-Methyl-<br>pyrrolidinone                     | 0.30                           | <<1<br>(<0.5)            | 0.22    | 0.06     | 0.20     | 0.07 |

\*The image was formed on the photosensitive material after the storage stability test.

\*\*The pKa of the acidic proton of the benzotriazole was 8.57.

\*\*\*The pKa of the acidic proton of the tetrazole was 4.9.

|                                                    |        |    |
|----------------------------------------------------|--------|----|
| Polymethyl methacrylate                            | 1.2 g  | 50 |
| Methyl ethyl ketone                                | 16.3 g |    |
| Phthalazinone                                      | 0.28 g |    |
| 2,2'-Methylenebis(6-tert-butyl-<br>4-methylphenol) | 0.70 g |    |

55 Each of the photosensitive materials thus obtained which were non-photosensitive under normal light conditions was preliminarily heated at 110° C. for 1 second in a dark room, and then exposed to light from a 300

## EXAMPLE 8

The same procedures as described in Example 7 were repeated except that 0.10 g of N-iodophthalimide was used instead of the iodine molecule.

The maximum optical densities and the minimum optical densities of the images thus formed and those of the images formed after the same storage stability test as in Example 7 are shown in Table 7 below.

Table 7

| Run<br>No. | Nitrogen-containing<br>Organic Base<br>(g) | Optical Density of Image |         |          |          |      |
|------------|--------------------------------------------|--------------------------|---------|----------|----------|------|
|            |                                            | Maximum                  | Minimum | Maximum* | Minimum* |      |
| 1          | Quinoline                                  | 0.30                     | 1.32    | 0.06     | 1.27     | 0.07 |
| 2          | 2-Methylquinoline                          | 0.30                     | 1.16    | 0.07     | 1.09     | 0.07 |
| 3          | 5-Methylquinoline                          | 0.30                     | 1.30    | 0.06     | 1.29     | 0.07 |
| 4          | 3-Chloroquinoline                          | 0.30                     | 1.09    | 0.06     | 1.09     | 0.07 |
| 5          | Pyridine                                   | 0.30                     | 1.24    | 0.06     | 1.22     | 0.08 |
| 6          | α,α'-Dipyridyl                             | 0.30                     | 1.00    | 0.06     | 1.01     | 0.07 |

Table 7-continued

| Run No.             | Nitrogen-containing Organic Base (g) | Optical Density of Image |         |          |          |
|---------------------|--------------------------------------|--------------------------|---------|----------|----------|
|                     |                                      | Maximum                  | Minimum | Maximum* | Minimum* |
| 7                   | 2-Tert-butyl pyridine                | 0.30                     | 1.35    | 0.07     | 1.33     |
| 8                   | 2,2-Diisopropyl- pyridine            | 0.30                     | 1.08    | 0.06     | 1.01     |
| 9                   | 3-Acetylpyridine                     | 0.30                     | 1.41    | 0.06     | 1.35     |
| 10                  | Primingine                           | 0.30                     | 1.27    | 0.06     | 1.29     |
| 11                  | 4-Methylpyrimidine                   | 0.20                     | 1.11    | 0.06     | 1.10     |
| 12                  | Phthalazine                          | 0.10                     | 1.52    | 0.07     | 1.51     |
| 13                  | Pyrazole**                           | 0.10                     | 1.33    | 0.05     | 1.33     |
| 14                  | 3-Methylpyrazole                     | 0.10                     | 1.34    | 0.06     | 1.35     |
| 15                  | Benzimidazole***                     | 0.30                     | 1.38    | 0.06     | 1.41     |
| Comparative Run No. |                                      |                          |         |          |          |
| 1                   | None                                 | —                        | 0.10    | 0.06     | 0.10     |
| 2                   | Benztriazole                         | 0.30                     | 0.27    | 0.06     | 0.20     |
| 3                   | Tetrazole                            | 0.30                     | 0.29    | 0.06     | 0.20     |
| 4                   | 3,6-Diazaindole****                  | 0.30                     | 0.41    | 0.06     | 0.38     |

\*The image was formed on the photosensitive material after the same storage stability test as in Example 7.

\*\*The pKa of the acidic proton of the pyrazole was 14.0.

\*\*\*The pKa of the acidic proton of the benzimidazole was 12.3 and the pKa of the conjugate acid was 5.53.

\*\*\*\*The pKa of the acidic proton of the 3,6-diazaindole was 10.88 and the pKa of the conjugate acid was 6.1.

## EXAMPLE 9

## 25

The same procedures as described in Run Nos. 1 to 5, 7 to 9 and 11 and Comparative Run Nos. 1 and 4 in Example 1 was repeated except that 0.12 g of N-iodosuccinimide was used instead of the iodine molecule and that the thickness of the first layer was 3 $\mu$  instead of 4 $\mu$  and the total thickness of the first and the second layers was 6 $\mu$  instead of 7 $\mu$ .

The maximum optical densities and the minimum optical densities of the images thus formed and those of the images after the same storage stability test as in Example 1 are shown in Table 8 below.

30  
35

## EXAMPLE 10

The same procedures as described in Run Nos. 1 to 5 and Comparative Run No. 1 in Example 1 were repeated except that 0.12 g of N-bromophthalazinone was used instead of the iodine molecule and that 0.28 g of phthalimide was used instead of the phthalazinone and the heat-development was carried out at 120° C. for 10 seconds.

The maximum optical densities and the minimum optical densities of the images thus formed and those of the images after the same stability test as in Example 1 are shown in Table 9 below.

Table 8

| Run No.             | Nitrogen-containing Organic Base (g) | Optical Density of Image |         |          |          |
|---------------------|--------------------------------------|--------------------------|---------|----------|----------|
|                     |                                      | Maximum                  | Minimum | Maximum* | Minimum* |
| 1                   | Pyridine                             | 0.30                     | 1.32    | 0.08     | 1.27     |
| 2                   | Quinoline                            | 0.30                     | 1.29    | 0.08     | 1.28     |
| 3                   | Isoquinoline                         | 0.30                     | 1.33    | 0.08     | 1.29     |
| 4                   | Phthalazine                          | 0.05                     | 1.51    | 0.08     | 1.50     |
| 5                   | Quinazoline                          | 0.60                     | 1.40    | 0.08     | 1.38     |
| 6                   | Pyridazine                           | 0.30                     | 1.41    | 0.07     | 1.42     |
| 7                   | Primingine                           | 0.30                     | 1.33    | 0.08     | 1.31     |
| 8                   | Quinoxaline                          | 0.60                     | 1.37    | 0.08     | 1.33     |
| 9                   | Pyrazole                             | 0.05                     | 1.34    | 0.08     | 1.30     |
| Comparative Run No. |                                      |                          |         |          |          |
| 1                   | None                                 | —                        | 0.16    | 0.07     | 0.13     |
| 2                   | Pyrrolidine                          | 0.05                     | 1.39    | 0.08     | 1.36     |

\*The image was formed on the photosensitive material after the same stability test as in Example 1.

Table 9

| Run No.             | Nitrogen-containing Organic Base (g) | Optical Density of Image |         |          |          |
|---------------------|--------------------------------------|--------------------------|---------|----------|----------|
|                     |                                      | Maximum                  | Minimum | Maximum* | Minimum* |
| 1                   | Pyridine                             | 0.20                     | 1.12    | 0.07     | 1.10     |
| 2                   | Quinoline                            | 0.20                     | 1.23    | 0.07     | 1.17     |
| 3                   | Isoquinoline                         | 0.20                     | 1.21    | 0.06     | 1.22     |
| 4                   | Phthalazine                          | 0.20                     | 1.08    | 0.06     | 1.09     |
| 5                   | Quinoxaline                          | 0.20                     | 1.19    | 0.06     | 1.18     |
| Comparative Run No. |                                      |                          |         |          |          |
| 1                   | None                                 | —                        | 0.11    | 0.06     | 0.11     |

\*The image was formed on the photosensitive material after the storage stability test as in Example 1.

## EXAMPLE 11

A silver stearate suspension was prepared in the same manner as in Example 1 except that the same amount of silver stearate as the silver behenate was used instead of the silver behenate.

An emulsion having the composition as set forth below was prepared by mixing each of its ingredients in the order described therein with stirring and coated on a sheet of art paper, and then dried.

| Composition                                                      |        |
|------------------------------------------------------------------|--------|
| Silver stearate suspension                                       | 12.0 g |
| Polyvinyl butyral                                                | 3.0 g  |
| Methyl ethyl ketone                                              | 12.0 g |
| N-Bromosuccinimide                                               | 0.05 g |
| Mercuric acetate                                                 | 0.01 g |
| Maleinimide                                                      | 0.5 g  |
| Nitrogen-containing organic base as shown below*                 | 0.1 g  |
| 2,6-Bis(2'-hydroxy-3'-tert-butyl-5'-methylbenzyl)-4-methylphenol | 1.5 g  |

- \*(1) Phthalazine
- (2) Pyridine
- (3) Quinoline
- (4) Isoquinoline
- (5) Quinazoline
- (6) Cinnoline
- (7) None

Each of the photosensitive materials thus obtained was preliminarily heated at 100° C. for 5 seconds with a hot roll, and then exposed to light from a 500 watt tungsten lamp for one eighth of second through a mask film, and subsequently heated at 130° C. for 2 seconds with a hot roll to develop a negative image.

The image formed on the photosensitive material not containing the nitrogen-containing organic base was barely observed in yellow color.

On the other hand, the image formed on the photosensitive material containing the phthalazine, pyridine, quinoline, isoquinoline, quinazoline or cinnoline was dark and clear, and the storage stability of the photosensitive was excellent.

While the invention has been described in detail and with reference to specific embodiments thereof, it will be apparent to one skilled in the art that various changes and modifications can be made therein without departing from the spirit and scope thereof.

What is claimed is:

1. In a heat developable photosensitive material comprising:

- (a) an organic silver salt oxidizing agent;
- (b) a halogen molecule or an organic haloamide compound; and
- (c) a reducing agent for silver ion; the improvement which comprises incorporating therein (d) at least one nitrogen-containing organic base selected from the group consisting of pyridine, quinoline, isoquinoline, acridine, phenanthridine, pyridazine, pyrimidine, pyrazine, cinnoline, phthalazine, quinazoline, quinoxaline, phenazine, m-, o-, p-phenanthroline, pteridine, pyrazole, imidazole, benzimidazole, 2-chloropyridine, 3-chloropyridine, 2-bromopyridine, 3-bromopyridine, 2-methylpyridine, 3-methylpyridine, 4-methylpyridine, 2,6-diisopropylpyridine, 2-isopropylpyridine, 2-tert-butylpyridine, 3-phenylpyridine, 2,6-di-tert-butylpyridine, 3-acetylpyridine,  $\alpha\alpha'$ -dipyridyl,  $\beta\beta'$ -dipyridyl,  $\gamma\gamma'$ -dipyridyl, 5-nitro-1,10-phenanthro-

line, 2-methylquinoline, 3-methylquinoline, 4-methylquinoline, 2-chloroquinoline, 4-chloroquinoline, 2-methoxyisoquinoline, 4-methylpyrimidine, 2-dimethylaminopyrimidine, 2-methoxyquinazoline, 2-methylquinoxaline, 1-methylpyrazole and 2-methylpyrazole, in an amount of about 0.001 mole to about 1 mole per mole of the organic silver salt oxidizing agent (a).

2. The heat developable photosensitive material of 10 claim 1, wherein the halogen molecule is at least one compound selected from the group consisting of molecular iodine, molecular bromine, iodine monochloride, iodine trichloride, iodine bromide and bromine chloride.

15 3. The heat developable photosensitive material of claim 1, wherein the halogen molecule is molecular iodine.

4. The heat developable photosensitive material of 20 claim 1, wherein the organic haloamide compound is at least one compound selected from the group consisting of N-chlorosuccinimide, N-bromosuccinimide, N-iodosuccinimide, N-chlorophthalimide, N-bromophthalimide, N-iodophthalimide, N-chlorophthalazinone, N-bromophthalazinone, N-iodophthalazinone, N-chloroacetamide, N-bromoacetamide, N-iodoacetamide, N-chloroacetylalide, N-bromoacetylalide, N-iodoacetylalide, 1-chloro-3,5,5-trimethyl-2,4-imidazolidinedione, 1-bromo-3,5,5-trimethyl-2,4-imidazolidinedione, 1,3-di-chloro-5,5-dimethyl-2,4-imidazolidinedione, 1,3-dibromo-5,5-dimethyl-2,4-imidazolidinedione, 1,3-diiodo-5,5-dimethylimidazolidinedione, N,N-dichlorobenzene sulfonamide, N,N-dibromobenzene sulfonamide, N-bromo-N-methylbenzenesulfonamide, N-chloro-N-methylbenzenesulfonamide, N,N-diiodobenzene sulfonamide, N-iodo-N-methylbenzenesulfonamide, 1,3-dichloro-4,4-dimethylhydantoin, 1,3-dibromo-4,4-dimethylhydantoin, and 1,3-diiodo-4,4-dimethylhydantoin.

25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 91